

Aug. 20, 1946.

S. W. FERRIS

2,406,210

METHOD OF CONTROLLING WAX SWEATING

Filed Oct. 19, 1942



Attest

John G. Buly  
Frank M. Williams

Inventor

Seymour W. Ferris  
By Robert E. Birch  
Attorney

## UNITED STATES PATENT OFFICE

2,406,210

METHOD OF CONTROLLING WAX  
SWEATINGSeymour W. Ferris, Mount Holly, N. J., assignor to  
The Atlantic Refining Company, Philadelphia,  
Pa., a corporation of Pennsylvania

Application October 19, 1942, Serial No. 462,653

7 Claims. (Cl. 196—20)

1

The present invention relates to the sweating of oily wax to reduce the oil content thereof, and relates more particularly to improvements in controlling the sweating of such wax.

An object of this invention is to control wax sweating in such a manner as to produce high yields of wax of reduced oil content without substantial loss of desirable wax in the sweat oil.

A further object of this invention is the application to wax sweating of a control method in which the control factors may be determined easily and rapidly, and the results thus obtained immediately applied in controlling the sweating operation.

The sweating of oily wax is generally carried out for the purpose of removing oil from the wax, and has long been used for the deoiling of paraffin wax, such as slack wax obtained from the pressing of paraffin distillates. Slack wax usually contains from 25% to 40% by weight of oil, and from such oily wax is made a variety of wax products of reduced oil content. For example, a commercial product such as scale wax contains from 8% to 10% of oil, whereas fully refined paraffin wax contains less than about 4% of oil, and high tensile strength paraffin wax contains less than 1.5% of oil, all of the oil contents being determined by treatment with ethylene dichloride as described more fully hereinafter.

Heretofore, in the sweating of oily wax, it has been very difficult to judge when the oil has been completely removed, or removed to the desired extent, from the wax remaining in the sweating pans. This difficulty arises from the fact that it is practically impossible to obtain a sample representative of all of the wax remaining in the sweating pans, and in addition, the determination of the oil content of the sweated wax by a selective solvent method is time-consuming. When more than one cycle of sweating is employed for the production of a fully sweated wax, there is a greater likelihood that the final product will be substantially oil-free, but when single cycle sweating is carried out, the determination of the proper time to terminate the sweating becomes more important, since stopping too soon results in incomplete oil removal and low tensile strength, and if each run is carried far enough to insure the production of high tensile strength wax, the average yield of the wax will be reduced.

It has been found that one of the most distinctive properties of a wax is the relationship between its melting point and its refractive index measured at some temperature above its melt-

2

ing point. For convenience, the melting point is determined in accordance with A. S. T. M. Method D87-37 "Melting point of paraffin wax," and the refractive index is measured at 176° F. in a suitable refractometer.

In accordance with the present invention, use is made of the relationship of the melting point and refractive index of the sweated wax and the sweat stream in controlling the duration of the sweating operation. More specifically, a sample of an oily wax is experimentally sweated by slowly raising the temperature of the mixture, and successive samples of the material sweated from the mixture, i. e., the sweat stream, are taken. The melting point, refractive index, and oil content of each of the samples is determined, and the oil content of the sweated wax may also be determined at each interval at which a sweat stream sample is taken. From the refractive index-melting point relationship of the sweat stream samples and the oil contents of the sweat stream and sweated wax samples, it is thus possible to determine experimentally the point at which sweating should be stopped in order to obtain a final wax having a desired oil content. The results thus determined experimentally for a given wax stock may then be applied directly to the control of a large scale commercial sweating operation. For example, a given wax stock is sweated on large scale and successive sweat stream samples are taken. The melting point and refractive index of each sample is determined as rapidly as the sample is taken from the sweat stream. When the refractive index-melting point relationship of a sweat stream sample is found to correspond to an experimentally determined value indicating a known oil content in the experimentally sweated wax or sweat stream sample, the large scale sweating operation is stopped and the resulting sweated wax will be found to have substantially the same oil content as the experimentally sweated wax. Thus, by simply determining the refractive index-melting point relationship of a sweat stream sample from a commercial sweating oven and comparing it with the refractive index-melting point relationship of sweat stream samples predetermined experimentally for sweated wax of known oil content, it is possible to control closely the large scale sweating of wax and to stop the sweating at exactly the proper time so that the wax is neither under-sweated nor over-sweated. Since the refractive index and melting point of the sweat stream samples are easily and rapidly deter-

minable, there is little or no lag in shutting down the sweating operation at the proper time.

The present invention may be further understood with reference to the accompanying drawing, which illustrates the relationship between the refractive index and melting point for sweat

Manufacturing Company, the durometer scale being calibrated from zero to 100. The 100 durometer reading indicates no penetration, while the zero reading indicates complete penetration. Tensile strength of the wax is given in lbs./square inch.

|   | Sweat stream      |               |                | Sweated wax   |                |                           |          |        |                     |
|---|-------------------|---------------|----------------|---------------|----------------|---------------------------|----------|--------|---------------------|
|   | R. I.,<br>176° F. | M. P.,<br>°F. | Percent<br>oil | M. P.,<br>°F. | Percent<br>oil | Weight per-<br>cent yield | Hardness |        | Tensile<br>strength |
|   |                   |               |                |               |                |                           | 86° F.   | 95° F. |                     |
| E | 1.4382            | 95            | 37.5           |               |                |                           |          |        |                     |
| F | 1.4350            | 99            | 28.5           |               |                |                           |          |        |                     |
| G | 1.4291            | 109           | 14.9           |               |                |                           |          |        |                     |
| H | 1.4280            | 115           | 8.6            | 126.6         | 2.0            | 29.8                      |          |        |                     |
| I | 1.4273            | 120           | 4.1            | 129           | 1.0            | 23.2                      | 30       | 0      | 132                 |
| J | 1.4275            | 127.5         | 1.1            | 133.5         | 0.3            | 6.3                       | 90       | 30     | 378                 |

stream samples from a commercial slack wax, and the correlation of such relationship with the oil content of the sweat stream samples and of the sweated wax.

Referring to the drawing, in which refractive index is plotted against melting point, the lines AB and CD represent the limits within which lie the majority of the hydrocarbons present in substantially oil-free waxes. The pure straight-chain paraffin hydrocarbons will be found to lie along the line AB, whereas the substantially oil-free waxes may lie anywhere within the area defined by AB and CD. The equation for the line AB is  $n=1.3950+.000242T$ , and the equation for the line CD is  $n=1.3793+.0004T$ , "n" being the refractive index at 176° F., and "T" being the A. S. T. M. melting point °F.

Upon the drawing is also plotted a curve defined by the points E, F, G, H, I, and J, representing the refractive index-melting point relationships of successive sweat stream samples from an experimentally sweated heavy paraffin slack wax having an initial oil content of 33.4% by weight and a melting point of 106° F. The oil content of the slack wax, as well as that of the sweat stream samples and sweated wax, was determined by the following method.

25 grams of oily wax is dissolved in ethylene dichloride and made up to 500 cc. at room temperature (75° F.), the solution is then cooled with stirring to 5° F. and filtered at such temperature through rapid filtering qualitative filter paper. The wax on the filter is then thoroughly washed with ethylene dichloride at 5° F., and an aliquot portion of the filtrate (100 cc.), measured at room temperature (75° F.) is transferred to a weighed evaporating dish, and the ethylene dichloride is removed by evaporation at 220° F., using a current of air to sweep out the vapors. A partial vacuum may be applied when most of the ethylene dichloride has been removed, in order to facilitate the removal of the last traces of the solvent. The oil residue is weighed and multiplied by a factor to correct for the aliquot portion of the ethylene dichloride filtrate employed. The corrected value is the weight per cent of oil in the oil wax sample.

In the following table are given the refractive indices (R. I.), melting points (M. P.), and oil contents for the sweat stream samples E, F, G, H, I, and J, as well as the melting points, oil contents, yields, hardness, and tensile strength for the sweated waxes when the sweating was stopped at points H, I, and J. The hardness was determined by means of an instrument known as a durometer supplied by the Shore Instrument

Referring again to the drawing, the constituents of a hydrocarbon wax, such as a substantially oil-free paraffin wax, have refractive index-melting point relationships which fall within the area defined by the lines AB and CD. Liquid constituents of paraffin distillate, however, exhibit relatively high refractive indices, and when the refractive index-melting point relationship of the first sweat stream sample is found to lie, for example, at point E, it is immediately known that considerable oil is present. When the slack wax is subjected to further sweating, however, the sweat stream shows progressively less oil and therefore the points will be found to move to the left as indicated at F, G, H, and I on the drawing. At such time as the quantity of oil in the sweat stream samples has reached a very low value, for example, point I, the successive points will no longer proceed to the left of the drawing but will rise, due to the increasing melting points, and inasmuch as such samples are approaching the composition of substantially pure wax (point J), the points will roughly parallel the line AB. When such condition is reached, the wax remaining in the sweating pans is substantially free of oil. For any particular wax stock, it may be determined experimentally how close the refractive index-melting point value of the sweat stream must approach the line AB before the sweated wax remaining in the pans is of desired quality. Each wax stock has a particular curve of its own, and the position of the curve on the accompanying drawing may change as either the boiling range or the source of the wax distillate, and therefore the wax stock, varies.

In order to produce from a slack wax stock having an oil content of from 25% to 40% by weight, a commercial grade of scale wax having an oil content of 8% to 10%, it has been found that the refractive index-melting point relationship of the sweat stream should fall within the limits defined by lines having the equations  $n=1.3998+.000242T$  and  $n=1.4003+.000242T$ . For the production of a fully refined paraffin wax of commercial grade having an oil content of less than 4% by weight, for example, 1.5% to 4%, the refractive index-melting point relationship of the sweat stream should fall within the limits defined by lines having the equations

$$n=1.3978+.000242T \text{ and } n=1.3983+.000242T$$

And for the production of high tensile strength wax containing less than about 1.5% of oil, and preferably less than 1% of oil, the refractive index-melting point relationship of the sweat stream should fall within the limits defined by

lines having the equations  $n=1.3964+0.000242T$  and  $n=1.3969+0.000242T$ .

In another aspect of the present invention, it has been found that the refractive index of the sweat stream is, per se, a valuable guide in indicating the point at which sweating should be terminated, particularly in the production of waxes of exceedingly low oil content, i. e., less than about 1% by weight of oil. By determining the minimum refractive index of the sweat stream and then terminating sweating when such value is reached, the resulting sweated wax will contain little or no oil. Referring to the drawing, it will be seen that the minimum refractive index of the sweat stream is reached at a point 10 between I and J, and that the oil content of the sweated wax when the sweating was stopped at I was about 1%. By terminating the sweating at the minimum refractive index between I and J, a somewhat higher yield of low oil content 20 wax would be obtained than by continuing the sweating to the point J.

The large scale or commercial sweating operations referred to herein may be carried out in the conventional sweating ovens well known to 25 those skilled in the art, wherein the oily wax stock is introduced into sweating pans and the temperature of the wax then slowly but progressively raised to effect sweating and removal of the sweatable constituents of the wax.

I claim:

1. The method of sweating oily wax to produce substantially oil-free wax, which comprises sweating an oily wax, determining the refractive indices and the melting points of successive samples of the sweat stream, and terminating the sweating of the wax when a sweat stream sample exhibits a melting point higher than that of the preceding sample, and a refractive index at least as great as that of said preceding sample.

2. The method of reducing the oil content of oily wax, which comprises subjecting said oily wax to sweating, and terminating the sweating of the wax when the refractive index of the sweat stream attains a minimum value.

3. The method of reducing the oil content of oily wax, which comprises subjecting said oily wax to sweating, and terminating the sweating of the wax when the relationship between the refractive index at 176° F. and the melting point in °F. of at least two successive samples of the sweat stream fall, on a plot of refractive index versus melting point, substantially parallel to the line represented by the equation

$$n=1.3950+0.000242T$$

where "n" denotes the refractive index and "T" denotes melting point in °F.

4. The method of reducing the oil content of oily wax, which comprises subjecting said oily wax to sweating, and terminating the sweating of the wax when the relationship between the refractive index at 176° F. and the melting point in °F. of a sweat stream sample falls, on a plot of refractive index versus melting point, within the lines defined by the equations

$$n=1.3964+0.000242T$$

and  $n=1.4003+0.000242T$ , where "n" denotes the refractive index and "T" denotes melting point in °F.

5. The method of producing a high tensile wax, which comprises subjecting an oily wax to sweating, and terminating the sweating of the wax when the relationship between the refractive index at 176° F. and the melting point in °F. of a sweat stream sample falls, on a plot of refractive index versus melting point, within the lines defined by the equations

$$n=1.3964+0.000242T$$

and  $n=1.3969+0.000242T$ , where "n" denotes the refractive index and "T" denotes melting point in °F.

6. The method of producing a refined wax, which comprises subjecting an oily wax to sweating, and terminating the sweating of the wax when the relationship between the refractive index at 176° F. and the melting point in °F. of a sweat stream sample falls, on a plot of refractive index versus melting point, within the lines defined by the equations  $n=1.3978+0.000242T$  and  $n=1.3983+0.000242T$ , where "n" denotes the refractive index and "T" denotes melting point in °F.

7. The method of producing scale wax, which comprises subjecting an oily wax to sweating, and terminating the sweating of the wax when the relationship between the refractive index at 176° F. and the melting point in °F. of a sweat stream sample falls, on a plot of refractive index versus melting point, within the lines defined by the equations  $n=1.3998+0.000242T$ , and

$$n=1.4003+0.000242T$$

where "n" denotes the refractive index and "T" denotes melting point in °F.

SEYMOUR W. FERRIS.